

J. T. OSLER.

## METHOD OF MAKING CHILLED ROLLS WITH STEEL CENTERS.

APPLICATION FILED DEC. 18, 1913.

1,132,611.

Patented Mar. 23, 1915.



FIG.3



## WITNESSES

J. T. Holmes  
Elbert Leedy

**INVENTOR**

INVENTOR

# UNITED STATES PATENT OFFICE.

JAY T. OSLER, OF CORAOPOLIS, PENNSYLVANIA.

## METHOD OF MAKING CHILLED ROLLS WITH STEEL CENTERS.

Specification of Letters Patent. Patented Mar. 23, 1915.

1,132,611.

Application filed December 18, 1913. Serial No. 807,469.

*To all whom it may concern:*

Be it known that I, JAY T. OSLER, resident of Coraopolis, in the county of Allegheny and State of Pennsylvania, have invented a new and useful Improvement in Methods of Making Rolls with Steel Centers, of which the following is a specification.

This invention relates to composite mill rolls and the method of making the same. Mill rolls, as a rule, are worked very close to their ultimate strength. The materials of which rolls are made are usually selected for their wearing qualities and their ability to take a good finish and not primarily for their strength. If it were not for this fact very few cast iron or high carbon steel rolls would be used, lower carbon steel or alloy steel rolls being preferable from the standpoint of strength. Cast iron mill rolls, however, are subjected to frequent variations in temperature, and the differences in expansion and contraction of the metal near the surface and along the core of the roll are frequently sufficient to rupture or crack the body of the roll. This is particularly true in the case of chilled cast iron rolls, which are very hard and are more liable to break or crack. It has been proposed to form chilled cast iron rolls by first placing a heated steel billet in a mold and then pouring molten cast iron around the same in such a manner as to secure a weld between the steel core and cast iron body. In such methods, however, it has been impossible to bring the heated billet and molten iron into contact with each other at the same temperature, or even at the best working temperature. The core cools rapidly while being carried from the heating furnace to the mold and while being introduced therewith and is usually considerably cooler than the molten iron when the latter is poured into the mold. Consequently, the center rapidly absorbs heat from the molten cast iron and quickly cools the same. This rapid cooling produces allotrophic changes in the structure of the cast iron and it becomes brittle and is liable to rupture under the heavy loads and varying temperature conditions encountered in use.

The present invention has for its object the production of a composite mill roll having a body formed of one metal, say, cast iron, either chilled or unchilled, and a core

or center welded thereto and formed of another metal of greater strength and toughness, for example, steel, whereby the roll as a whole is stronger and not so liable to break and also has a surface which has the desired wearing quality and will take a good finish.

Another object of the invention is the production of a composite roll having a core or center which at all times is under initial tension or stress, whereby in use of the roll the heat tends to equalize the tension or stress throughout the roll but never entirely relieves the same, which reduces the net destructive stresses set up by the varying temperatures to which the roll is subjected during the rolling operation.

Another object of the invention is to provide a method of forming a composite roll which can be carried out in such manner that the heated steel core and the molten cast iron for the body can be brought into contact with each other at substantially the same temperature, whereby both the core and body will weld and cool under the same conditions and will not transmit heat one to the other, thereby producing a roll of maximum strength and durability.

According to the present invention the mold is arranged to receive or to cooperate with a billet heating furnace, which may be portable by a crane or fixed to the mold. This furnace is arranged to hold the core or center for the roll and said core may be heated in an ordinary furnace and transferred to the portable heating furnace and carried therein to the mold, or it may be heated entirely in the portable furnace. The portable furnace is placed in position on the mold with the heated core therein and the latter is maintained at the proper temperature, say about 2200 degrees Fahrenheit, until the molten iron for forming the roll body is in the proper condition for pouring. The molten metal is heated slightly above the temperature of the heated core, say 2400 degrees Fahrenheit, and is then underteamed into the mold. When the proper quantity of molten metal has been run in, the heated core or center is lowered into the molten metal, preferably, although not necessarily, passing through cleaning devices to free the billet from scale and provide it with clean surfaces so that it will readily unite or weld with the molten metal.

Preferably, also, centering devices are provided so that when the core seats in the mold it need not be again moved, but will be perfectly central in the mold cavity and 5 surrounded on all sides with an equal thickness of molten metal. From the time of pouring the molten metal into the mold to the introduction of the heated core thereinto the molten metal gradually cools down until 10 at the time the core seats the core and the molten metal will be at substantially the same temperature, that is, the temperature of the core—about 2200 degrees. The core is preferably made somewhat longer than 15 actually necessary so that it sinks clear to the bottom of the mold by its own weight and will not be liable to float in the molten iron. The extra length at the ends of the core may afterward be cut off to trim the 20 roll down to proper shape and size.

The invention will be more readily understood by reference to the description herein-after, taken in connection with the accompanying drawings, wherein—

25 Figure 1 represents a sectional elevation of suitable apparatus for carrying out the method; Fig. 2 is a detail view on a larger scale, of the centering devices; Fig. 3 is a horizontal section on the line 3—3, Fig. 2; 30 and Fig. 4 is a sectional view of the finished roll.

The mold may be arranged for casting either chilled or unchilled rolls, and in the drawings is arranged for casting chilled rolls. It comprises the body chill 1 and neck sand portions 2, which are suitably clamped together and rest upon a base or bottom 3, the lower sand portion 2 being preferably formed with a conical depression 35 to receive the pointed end of the core or billet. The molten metal is introduced into the mold through a spout 4 which enters the bottom of the mold. Supported upon the upper end of the mold is a casing 5 within 40 which is located the centering rig for centering the core in the mold cavity. This centering rig comprises two superposed sets of pivoted arms 6, having counterweights 7 at their outer ends, and having their inner ends arranged to contact the core and center it as it is lowered into the mold. Each 45 set preferably comprises three or more centering fingers, and the fingers of the two sets are in staggered relation with each other, as shown in Fig. 3. The centering fingers may be arranged to completely surround the core, as fully described in my companion application for apparatus for 50 making composite rolls, filed of even date herewith, Serial No. 807,470, and not only center the same, but also free it from scale and clean its surface as it passes through so 55 that it will readily and completely weld or unite with the molten metal for forming the body. The upper end of the casing 5 is

preferably closed by a shield 9, which is in the form of a sliding gate arranged so that it may be moved into position to close the lower end of the heating furnace, as herein-after described, or withdrawn therefrom 70 when it is desired to lower the core into the mold.

The heating furnace is represented at 10, and preferably comprises a cylindrical casing or jacket 11 with a lining 11<sup>a</sup> of refractory material, such as fire brick or the like. The furnace is heated by means of any suitable number of burners 12, arranged in any manner. The lower end of the furnace rests upon the top of the casing 5 and is closed by 75 the gate 9 before referred to. The upper end of the furnace is preferably provided with any suitable means, such as the trunnions 14, by means of which it may be lifted and transported from place to place. 80

In use of the apparatus a core 15 is slowly heated up to the proper temperature. This may be done in an ordinary furnace, or directly in the portable furnace 10. In the former case the core is first heated in the 90 ordinary furnace to about the proper temperature and is then removed and placed in the portable furnace 10, which is then carried to and placed in position on top of the mold in the position shown in Fig. 1, where 95 the billet is finally heated to the proper temperature. In the second case the core is placed directly in the portable furnace, while in position on the mold, and is there heated to the proper temperature. It will, 100 of course, be understood that the core 15 may be made of any suitable material, but preferably is of soft or mild steel, possessing the proper degree of toughness and resiliency to withstand heavy strains without 105 breaking. The body 16 of the roll is formed of cast iron, which is heated in any suitable furnace or cupola to a little higher temperature than the core or center 15, say to about 110 2400 degrees. When in the proper condition the molten metal is poured into the spout 4 and underteemed into the mold. It immediately begins to transmit its heat to the chill 1 and to chill on its outer surface. Gate 9 is now withdrawn to open up the 115 lower end of the heating furnace 10. Center or core 15 is now lowered into the mold. Its lower end is conical or pointed, as at 17, and first strikes the inner ends of the upper set of arms 6 which swing outwardly on 120 their pivots and hold the core in central position. They also preliminarily scrape the core and free it from scale. The second set of arms next encounters the core and assists in cleaning and centering the same. 125 The core sinks until its pointed center seats in the conical depression in the sand portion 2 with the core in a central or axial position in the mold cavity. In sinking the core displaces the central or axial portion 130

of the molten metal, without affecting that along the sides of the mold cavity, and forces it up through the spout 4 and out through a side gate 18 into a suitable receptacle. By the time the core seats in the mold the molten metal is cooled down to practically the same temperature as the core. Both the core and body then begin to cool at substantially the same rate. The 10 chill 1 produces a hard chilled surface on the body of the roll and the high temperature produces an intimate weld or union between the body and core.

It will, of course, be understood that the 15 co-efficients of expansion of cast iron and steel are slightly different. Consequently, in cooling, the iron body 16 contracts a little less than the core, thereby placing the core under an initial tensile stress, which becomes more and more fixed and pronounced 20 as the roll cools down. Similarly, the iron body 16 is placed under slight longitudinal compression, due to the same difference in contraction. When the roll has completely 25 cooled the extra lengths at the ends of the core are cut off and the roll is turned down to final shape.

At normal temperatures the roll is in a 30 condition of internal strain, with the core under tensile stress. In use of the roll the surface or body heats up first and thereby expands and increases the stress on the core, which, however, is made of steel and is well able to withstand tensile stresses. As 35 the heat soaks into the roll and temperature conditions become more uniform the greater co-efficient of expansion of the steel core over the iron body relieves some of the strain, but the strain is never entirely relieved because the roll is never heated up to 40 the temperature at which it was cast. The hotter the roll becomes, however, the nearer it approaches a condition of no internal strain. In cooling the surface or body of 45 the roll cools first, but as the internal strain has never been entirely relieved contraction

of the body does not place the body under tension or the core under compression, but merely relieves a little more of the internal strain. As cooling goes on the core begins 50 to shrink until when normal conditions are finally reached the original internal stresses are again set up.

The composite roll described has the metal disposed therein in the best possible manner 55 to withstand the bad effects of expansion and contraction produced by the varying temperature conditions encountered in use. It is consequently very durable and is not liable to develop flaws, cracks or breaks, and, 60 moreover, has a cast iron surface which will take a very good finish.

What I claim is:—

1. The method of forming rolls in a mold, consisting in first pouring into said mold 65 cast iron to form the roll body and then lowering into the cast iron a heated mild steel core to form the roll center, and allowing said core and body to cool.

2. The method of forming composite rolls 70 in a mold, consisting in heating a steel core to form the roll center, pouring into said mold molten iron at a temperature above that of the heated steel core, lowering the core into the molten cast iron, and allowing 75 the core and cast iron to cool and weld together.

3. The method of forming composite rolls 80 in a mold, consisting in heating a core to form the roll center, heating molten cast iron to form the body to a temperature slightly above that of the heated core, pouring said molten metal into the mold, lowering the heated core into the molten metal, and allowing the same to cool. 85

In testimony whereof, I have hereunto set my hand.

JAY T. OSLER.

Witnesses:

ELBERT L. HYDE,  
GLENN H. LERESCHE